

Sept. 13, 1932.

E. H. SCHULZ ET AL

1,877,063

METHOD OF PRODUCING HARD ALLOYS

Filed May 8, 1930



Inventors:  
E. Hermann Schulz  
K. Lobbecke

By: Mauz & Cie  
5/11/75.

## UNITED STATES PATENT OFFICE

ERNST HERMANN SCHULZ, OF DORTMUND, AND KARL LÖBBECKE, OF RHEINHAUSEN,  
GERMANY, ASSIGNORS TO VEREINIGTE STAHLWERKE AKTIENGESELLSCHAFT, OF  
DUSSELDORF, GERMANY

## METHOD OF PRODUCING HARD ALLOYS

Application filed May 8, 1930, Serial No. 450,818, and in Germany March 26, 1929.

The alloys of the stellite type i. e. those based on an alloy containing cobalt, chromium, tungsten and carbon and, if desired, other additional metals such as molybdenum, 5 nickel, iron, manganese etc. have, as is well known, apart from other valuable properties a very high resistance to abrasion. For this reason they are used for manufacturing machine parts which are subjected to severe 10 abrasive wear. Their superiority over other materials, for example alloyed steels, which are intended for the same purpose, is a generally recognized fact. Moreover, it is known that by an alteration of the pouring and 15 cooling conditions the texture of these alloys may be influenced within certain limits. This has a certain bearing upon the properties of the finished alloys in as much as coarse grained castings are more brittle 20 than castings having a fine-grain structure. Beyond these discoveries no influence of the pouring conditions upon the properties of the finished castings has yet been ascertained and the fact that the texture of 25 these alloys is completely stable and cannot be changed by any kind of heat treatment, has always been considered to be a particularly important property of these alloys.

In contradistinction thereto the inventors 30 have found that the pouring conditions as well as a subsequent heat treatment are capable of changing within very wide limits especially the resistance to abrasion of these stellite-like alloys. It has been ascertained 35 that the highest resistance to abrasion regularly occurred when the castings contained graphite which, as a constituent of the texture, has heretofore been entirely unknown with stellites.

An example of the decrease in abrasion 40 shows the drawn curve of the annexed drawing. For comparison the scleroscope as well as the Brinell hardness are given, by the dotted and dashed curves respectively. It 45 has been found that the abrasion decreases already with a graphite content which is incapable of impairing the hardness.

Although the presence of graphite in stellite-like alloys has in itself been an entirely 50 novel feature, the discovery that the for-

mation of graphite could be enhanced in a similar manner as with ordinary pig iron was still more astonishing. According to the invention a high graphite content is being obtained first, as in the case of cast iron, by 55 greatly retarding the rate of solidification and cooling after the pouring operation by suitably controlling the casting temperature, the temperature, dimensions and composition of the mould, second by making the carbon 60 content as high as to cause part thereof to separate out in the form of graphite even with a more rapid cooling. Experience has shown that this is the case when the carbon content amounts to more than 2%. Finally, 65 the separation of the graphite may be brought about also in the solidified alloy by heating the pieces to a temperature of more than 700° C. and holding them at this temperature for a certain period of time, whereupon they will be cooled down very slowly. 70 The lower the annealing temperature, the more time will be necessary for the annealing operation. Thus various ways will be given to impart to alloys of the stellite 75 type a resistance to abrasion which is far superior to that heretofore known.

We claim:

1. A method of producing hard alloys of the stellite type on the basis of cobalt, 80 chromium, tungsten and not over 3.5% carbon, a part of which is present in the form of graphite, consisting in forming the alloy by combining the requisite alloy components, casting the alloy thus formed and cooling 85 with retarded velocity.

2. A method of producing hard alloys of the stellite type on the basis of cobalt, chromium, tungsten and carbon, a part of which is present in the form of graphite, 90 consisting in forming the alloy by combining the requisite alloy components, casting the alloy in superheated condition so that slow solidification takes place.

3. A method of producing hard alloys of the stellite type on the basis of cobalt, chromium, tungsten and carbon, consisting in forming the alloy by combining the requisite alloy components, casting the alloy, cooling 95 the alloy and converting the carbon into 100

graphite by heating the solidified alloy to a temperature above 700° C. and slowly cooling the heated alloy.

4. Hard alloy of the stellite type based on the components cobalt, chromium, tungsten, and containing 2% to 3.5% carbon, the essential part of which is transformed into graphite by a method of the type known for transforming carbon into graphite in the manufacture of cast iron.

5. Method of producing hard alloys of the stellite type on the basis of cobalt, chromium, tungsten and carbon, comprising solidifying the alloys in the usual manner, obtaining the formation of graphite by heating the alloy thus solidified to a temperature of more than 700° C. and then cooling the alloy at a relatively slow rate.

**20** ERNST HERMANN SCHULZ.  
KARL LÖBECKE.

**25****30****35****40****45****50****55****60****65**